

## UNITED STATES PATENT OFFICE

2,599,353

## STAINLESS EMULSIBLE GREASE

Jere C. Showalter, Baytown, Tex., assignor, by  
mesne assignments, to Standard Oil Develop-  
ment Company, Elizabeth, N. J., a corporation  
of Delaware

No Drawing. Application June 21, 1950,  
Serial No. 169,512

3 Claims. (Cl. 252—21)

1

The present invention is directed to a stain-  
less, emulsible grease composition which may  
be employed in pipe bending and wire drawing  
operations and the like.

The stainless, emulsible grease composition of  
the present invention comprises a composition  
having as major ingredients an alkaline base oil  
containing alkali metal petroleum sulfonates and  
a hydrocarbon in the lubricating oil boiling range  
having a viscosity at 100° F. of 75 to 500 SSU and  
a solid having lubricating properties selected  
from the class consisting of talc and mica and  
minor amounts of tall oil, a polyhydroxy alcohol,  
an oil soluble corrosion inhibitor and a fatty acid.  
The solid having lubricating properties is em-  
ployed in a ratio of at least 1:2 to said alkaline  
base oil.

The composition of the present invention con-  
tains an alkaline base oil which includes an alkali  
metal petroleum sulfonate and a hydrocarbon in  
the lubricating oil boiling range having a viscosity  
of 75 to 500 SSU at 100° F. The alkaline base  
oil may be prepared preferably by exhaustively  
sulfonating with concentrated sulfuric acid a  
solvent extract of a lubricating oil fraction ob-  
tained from a naphthenic base crude, such as a  
lubricating oil fraction from a coastal crude. For  
example, a phenol extract of a lubricating oil  
fraction from a coastal crude having a viscosity  
of approximately 75 SSU at 100° F. may be ex-  
haustively treated with concentrated sulfuric  
acid, the sludge separated and the acid oil neu-  
tralized with caustic alkali, such as sodium hy-  
droxide and the neutralized oil, which may con-  
tain an excess of caustic alkali, finished by blow-  
ing with air to remove moisture. The finished  
base oil contains from 10% to 15% by weight  
of alkali metal petroleum sulfonates in addition  
to some excess caustic alkali with the remainder  
being unsulfonated oil.

The hydrocarbon oil and sulfonates which may  
contain a sufficient amount of caustic alkali to  
make the mixture alkaline may be prepared by  
admixing petroleum sulfonates, a hydrocarbon  
in the lubricating oil boiling range having the  
viscosity mentioned before and a small amount  
of a caustic alkali. The hydrocarbon oil ordi-  
narily boils in the lubricating oil boiling range  
and should have a viscosity of 75 to 500 SSU  
at 100° F. and should be relatively free of aromatic  
hydrocarbons. The alkaline base oil pro-  
duced, as mentioned before by exhaustively sul-  
fonating a phenol extract of a naphthenic lubri-  
cating oil fraction, may contain alkali metal  
petroleum sulfonates having molecular weights  
in the range from about 325 to 400. The alkaline  
base oil may be employed in the composition of  
the present invention in an amount in the range  
from 25% to 75% by weight with a preferred  
concentration in the range between 50% to 60%  
by weight. The petroleum sulfonates consist of

about 10% to 15% by weight of the alkaline  
base oil.

A composition in accordance with the present  
invention may contain the ingredients thereof  
in the proportions set out in the following table:

Table I

|                                     | Weight<br>Per Cent |
|-------------------------------------|--------------------|
| 10                                  |                    |
| Alkaline Base Oil.....              | 25 — 75            |
| Petroleum Sulfonate.....            | 2.5 — 11.5         |
| Oil.....                            | 22.5 — 63.5        |
| Tall Oil.....                       | 0.5 — 2.0          |
| Polyhydroxy Alcohol.....            | 0.5 — 2.0          |
| Cyclohexylamine.....                | 0.3 — 1.0          |
| Fatty Acid.....                     | 0.05 — 0.2         |
| 15                                  |                    |
| Talc or Mica Ratio to Base Oil..... | 1.2 — 2:1          |

The tall oil which is employed in my improved  
grease serves to impart adhesive powers to the  
20 mixture and may be employed in the grease com-  
position in an amount in the range from about  
0.5% to about 2% by weight, although it is prefer-  
ably employed in an amount in the range from  
0.5% to 0.6% by weight.

The polyhydroxy alcohol which imparts water  
emulsibility to the composition may be employed  
in an amount in the range from 0.5% to 2.0%  
by weight and preferably is employed in an  
amount in the range between 0.5% to 0.6% by  
30 weight. As examples of the polyhydroxy alcohol  
may be mentioned glycerine, propylene glycol,  
diethylene glycol, triethylene glycol, and the  
like. Other polyhydroxy alcohols may be used  
provided they are water soluble and miscible with  
35 the composition.

The corrosion inhibitor is preferably cyclo-  
hexylamine and should be present in a concen-  
tration of at least 0.3% by weight. The amount of  
40 corrosion inhibitor will depend on the par-  
ticular corrosion inhibitor employed but ordi-  
narily will not exceed 1% by weight of the com-  
position but preferably will be in an amount in  
the range of 0.4% and 0.5% by weight of the  
composition. As a general statement, it may be  
45 said that the corrosion inhibitor may be oil  
soluble. Examples of the oil soluble corrosion  
inhibitors are: pheylalphanaphthylamine, di-  
cyclohexylamine, isooctylphenolmethylamine,  
and the like.

The fatty acid is employed in the composition  
of the present invention to improve the lubricat-  
ing properties of the mixture. The fatty acid  
may also react with some of the excess alkali in  
the alkaline base oil and form, for example when  
50 stearic acid is employed, the stearate which im-  
proves the lubricating properties of the mixture  
and imparts increased bearing strength and acts  
as a soap or emulsifying agent to allow the im-  
proved grease to be removed by washing the sur-  
55 face, to which it is applied, with water. Ordin-  
arily the concentration of the fatty acid will  
60

be in the range from 0.05% to 0.2% by weight of the composition. Preferably it will be used in a concentration in the range from 0.09% to 0.1% by weight. Stearic acid is the preferred fatty acid but other fatty acids and fatty acid-containing materials may be used in lieu of stearic acid. For example, lard oil, oleic acid, palmitic acid, lauric acid, wool, fatty acids, tallow oil, linoleic acid and the like may be used.

The other major component of the composition of the present invention is a solid having lubricating properties selected from the class consisting of talc and mica. The amount of the solid having lubricating properties is dependent on the desired viscosity of the improved grease but generally the solid may be present in a concentration of about 33%. Stating this otherwise, the ratio of the solid such as talc or mica to the alkaline base oil should be at least 1:2 and generally should not exceed about 70% by weight of the composition or a ratio of 2:1 with respect to the alkaline base oil. If too much of the solid, such as talc or mica is used, the grease is very viscous so that the upper limit of the solids concentration depends on the viscosity of the grease desired. A grease composition which has been used commercially in bending pipe having large diameters is given in the following table:

Table II

| Compound               | Weight<br>Per Cent |
|------------------------|--------------------|
| Alkaline Base Oil..... | 60.23              |
| Tall Oil.....          | 0.62               |
| Diethylene glycol..... | 0.62               |
| Cyclohexylamine.....   | 0.44               |
| Stearic Acid.....      | 0.09               |
| Talc.....              | 38.00              |

The grease having the foregoing composition is successfully used in bending pipe in a large petroleum refinery. Equipment used for bending pipe of large diameter operates by holding the pipe to be bent adjacent to a large circular wheel while applying a block to the surface of the pipe opposite the pipe surface in contact with the wheel. The pipe and the wheel are slowly rotated with respect to one another. A close fitting, highly polished metal plug is placed in the pipe and travels inside the pipe just ahead of that portion of the pipe that is being bent, thus preventing the formation of wrinkles in the inner portion of the bend. The plug travels through the pipe ahead of the bend by virtue of the pressure exerted upon it by the attempt of that portion of the pipe which is being bent to collapse. In order for this plug to travel smoothly inside the pipe, it is necessary that the inner surface of the pipe be well lubricated. Ordinary oil will not suffice for this purpose because the heat caused by the bending operation makes the oil so fluid that it runs entirely to the lower surface of the pipe, thus leaving large areas of the pipe insufficiently lubricated. The usual preparation used for this lubrication is a grease which is moderately viscous at room temperature and which contains large quantities of graphite. This grease is sprayed on the inner surface of the pipe by means of a suitable moving spraying device and the plug is then inserted through the open end of the pipe and slid over this lubricated surface to 70 the point at which the bend is to be started. When the bending operation is complete, the plug and excess grease are removed. This grease, by virtue of the large quantity of graphite contained therein, is very messy to handle and difficult to 75

clean from the equipment and the operator and, therefore, unsatisfactory. In addition, when it is wiped from the plugs before they are stored, it leaves the highly polished surface of the plugs exposed to the air which causes them to corrode unless they are protected by means of a compound which must be coated over them until they are again to be used.

The composition of the present invention which includes a solid which does not soil surfaces with which it comes in contact serves to give the needed viscosity to the lubricating composition and furthermore it contains ingredients which allow it to be readily removed by washing with water thus making it easy to clean the metal plugs employed in such pipe bending operations. The presence of the corrosion inhibitor prevents rusting of the surfaces which have been treated with the grease and protects them from corroding during storage periods.

The composition of the present invention has been accepted commercially in pipe bending operations due to its stainless qualities and ease of removal by virtue of its eliminating the necessity of employing graphite and by virtue of its being readily soluble with water.

The nature and objects of the present invention having been fully described and illustrated, what I desire to claim as new and useful and to secure by Letters Patent is:

1. A stainless, emulsible grease composition which comprises 25% to 75% by weight of a base oil containing alkali metal petroleum sulfonates in an amount in the range between 10% and 15% by weight of said base oil, the remainder being a hydrocarbon in the lubricating oil boiling range, 0.5% to 2.0% by weight tall oil, 0.5% to 2.0% by weight of a polyhydroxy alcohol, 0.3% to 1% by weight of an oil soluble corrosion inhibitor, 0.05% to 0.2% by weight of a fatty acid, and a solid having lubricating properties selected from the class consisting of talc and mica in a ratio in the range between 1:2 and 2:1 to said base oil.

2. A stainless, emulsible grease composition which consists of about 60% by weight of a base oil containing alkali metal petroleum sulfonates in an amount in the range between 10% and 15% by weight of said oil and the remainder a hydrocarbon oil having a viscosity at 100° F. of 75 to 500 SSU, about 0.6% by weight tall oil, about 0.6% by weight diethylene glycol, about 0.4% by weight cyclohexylamine, about 0.1% by weight stearic acid and about 38% by weight of a solid having lubricating properties selected from the class consisting of mica and talc.

3. A composition in accordance with claim 2 in which the hydrocarbon oil is substantially free of aromatic hydrocarbons.

JERE C. SHOWALTER.

#### REFERENCES CITED

The following references are of record in the file of this patent:

#### UNITED STATES PATENTS

| Number    | Name         | Date          |
|-----------|--------------|---------------|
| 1,617,455 | Montgomery   | Feb. 15, 1927 |
| 1,781,607 | Stamberg     | Nov. 11, 1930 |
| 1,817,599 | Adams et al. | Aug. 4, 1931  |
| 2,112,632 | Montgomery   | Mar. 29, 1938 |
| 2,444,271 | Smith        | June 29, 1948 |
| 2,490,949 | De Lorenzo   | Dec. 31, 1949 |

#### FOREIGN PATENTS

| Number  | Country | Date          |
|---------|---------|---------------|
| 660,799 | France  | Feb. 25, 1929 |